

Sept. 24, 1963

J. T. MAYHEW

3,104,981

## HOT DIP METAL COATING METHOD

Filed Nov. 22, 1960



FIG. I



**FIG. 3**



FIG. 4

INVENTOR.  
JOHN T. MAYHEW  
BY *Stanley & O'Neil*  
ATTORNEY

1

3,104,981

**HOT DIP METAL COATING METHOD**  
John T. Mayhew, Toronto, Ohio, assignor to National  
Steel Corporation, a corporation of Delaware  
Filed Nov. 22, 1960, Ser. No. 71,909  
2 Claims. (Cl. 117—46)

The invention is concerned generally with hot-dip coating and more particularly with a method for producing an even coating on heavy coated flat rolled products.

In the hot-dip coating of flat rolled products, such as hot-dip galvanizing, considerable difficulty has been experienced with draping of the coating when a heavy coating is applied. For example, in the continuous hot-dip galvanizing wherein a coating of about 1.5 ounces per square foot of the product is applied, the molten metal will run at frequent intervals along the surface of the product. Visually the running or draping of the molten galvanize coating has the same appearance as that occurring when a too heavy brush stroke of wet paint is applied to a wall. This draping of the molten coating appears frequently, usually at less than two foot intervals longitudinally and less than 1 foot intervals laterally along the surface of the product. In solidifying, the run or drape presents an uneven, unattractive surface.

Uneven galvanize coating has other disadvantages in addition to its appearance. The draping actually removes coating from the product so that the valleys formed are below coating specifications. Correction of draping has long been a problem in the hot-dip galvanizing industry. All previously known solutions employed a process known as puddling. In this process, streams of compressed air were blown vertically upward onto the surface of the flat rolled product in a direction opposite to the direction of drape. If the air streams were properly positioned and at frequent enough intervals, a fair job could be done in minimizing the draping effect. Actually only the heaviest draping was smoothed over and the coating was moved by the air blasts so that the problem of uneven coating of the product still remained. Poor puddling resulted in splattering of the metal and wasted product. Puddling, even at its highest efficiency, is not adequate to the job as it is merely a remedial process rather than a preventative process. A significant part of the invention was the discovery and analysis of the source of the problem; a novel preventative process resulted therefrom.

In explaining the invention reference will be had to the accompanying drawings in which:

FIG. 1 is a side view of hot-dip coating apparatus;

FIG. 2 is a frontal view of the apparatus of FIG. 1;

FIG. 3 is an enlarged view of a portion of hot-dip coating apparatus; and

FIG. 4 is an enlarged view of a portion of coating apparatus employing the invention.

Referring to FIG. 1, in hot-dip galvanizing a flat rolled product 10 is introduced into a molten bath 11 through a controlled atmosphere chute 12. The flat rolled product is at a temperature above that of the molten bath and maintains the bath molten. The bath is normally zinc base with aluminum additions to suppress zinc-iron alloying.

The product travels downwardly around submerged roll 14 and then upwardly toward exit means which also function as coating control means. Coating control is effected by coating rolls 15 and 16; with the level of the molten bath 11, the pressure between the rolls 15 and 16, and the number of circumferential grooves present on the rolls determining the coating thickness.

After exit from the molten bath through the coating rolls 15 and 16 the coated product 17 travels upwardly into cooling towers (not shown). Normally the coating begins to solidify at about 8 to 15 feet above the nip of

2

the coating rolls, the distance varying with the temperature employed, the gauge of the base metal being coated, and the coating thickness. Before solidification some galvanized coatings above one ounce per square foot of product, and in all cases where galvanized coatings above about 1.5 ounces per square foot of product are applied, the draping effect described earlier takes place.

The invention includes the discovery of causes for the aforescribed draping of molten coatings in hot-dip coating practice. As the coated flat rolled product 17 moves upwardly through the coating rolls 15 and 16, molten metal accumulates above the nip 21 of the rolls 15 and 16 in crevices 22 and 23, existing on either side of the product between the coated flat rolled product 17 and the adjacent coating roll. The metal in the crevices 22 and 23 takes on a rotary motion because of the movement of the coated product 17 and the coating rolls 15 and 16 so that beads of metal 26 and 27 are formed in each crevice. The bead of metal in each crevice due to the relative motion between it and the coated product 17 picks up additional metal from the coated product and grows with a "snowballing" effect. This pick up of metal from the surface of coated product is believed to be caused by the surface tension between the molten coating metal on coated product 17 and metal in the crevices 22 and 23 respectively. At periodic intervals, as metal accumulates along crevices 22 and 23 the cohesive force of a bead of metal is overcome and a heavy blob of metal is deposited on the product. As the product 17 travels upwardly the heavy blobs of metal start to drape and pull further coating from the product above the drape.

In accordance with the invention the build-up of metal in the crevices 22 and 23 and the deposition of such metal on the coated product 17 is prevented. This build-up and deposition of metal is prevented by blowing a gas downwardly into the crevices between the coated product 17 and the coating rolls 15 and 16. By properly selecting the direction of flow of gas into the crevices 22 and 23 the draping of molten coating is eliminated entirely. It is believed the gas reduces the surface tension between the beads of metal 26 and 27 and the coating on the product 17 allowing the metal to flatten in the crevice as shown in FIG. 4.

When coke oven gas is blown into the crevices it is ignited by the temperatures existing around the coating pot. It has been observed, however, that the draping effect is discontinued immediately upon the flow of the gas, prior to the ignition thereof, so that a flame is not necessary to the operation of the invention.

Referring to FIGS. 2 and 4 a gas is introduced into the crevices through the pipes 30 and 31 and flows with a high volume and low pressure. The gas after contact in the crevices flows outwardly toward the lateral edges of the coated product 17 and the coating rolls 15 and 16. By the use of a high volume-low pressure gas splattering of the metal is avoided, and the coating remains evenly distributed on the coated flat rolled product 17.

Suitable gases include compressed air, or inert gases such as nitrogen. It is preferred that the gas be hot, either heated or in the form of a flame to prevent chilling of the coating rolls 15 and 16. Therefore, when heated gas is used a temperature approaching that of the coating bath 11 is employed to prevent chilling of galvanizing material on the rolls and the fouling thereof. When coke oven gas, blast furnace gas, or their equivalent is used a normal yellow, low-temperature flame is satisfactory as undue heating of the rolls or coating material is not desired. It is emphasized that having heat present in the gas prevents chilling of the coating rolls.

Under normal circumstances a single gas outlet located centrally of the flat rolled product is sufficient. It is important that the direction of gas flow be substantially

vertically downward onto the molten metal in the crevices 22 and 23; such a path has the effect of flattening the molten metal in the crevices as shown in FIG. 4. Normally this flow path of the gas will be substantially parallel to the path of the exiting flat rolled product 17.

In a specific embodiment of the invention employing coke oven gas the following values were measured:

|                                                          |                       |         |
|----------------------------------------------------------|-----------------------|---------|
| Gas pressure, in pipe                                    | lbs./in. <sup>2</sup> | 2-3     |
| Gas pressure, between pipe and crevice                   | lb./in. <sup>2</sup>  | 1/4     |
| Gas volume                                               | ft. <sup>3</sup> /hr  | 300-500 |
| Temperature, thermo-couple after 35 minutes in the flame | °F                    | 1000    |

Summarizing the invention, the cause of molten coating drape in hot-dip, heavy coating of flat rolled product has been discovered and analyzed and a method devised for preventing draping in which a gas is blown downwardly into a crevice between the exiting flat rolled product and the coating control means along a path which is substantially parallel to the path of the exiting flat rolled product.

What is claimed is:

1. In continuous strip-steel hot-dip metal coating where-in a heavy galvanize coating weight is applied such that draping of the molten galvanize coating on the strip would normally occur, a method for preventing such draping of the molten coating comprising the steps of:

applying a galvanize coating to the continuous strip steel by passing the strip upwardly through a molten metal bath,

controlling the weight of the galvanize coating to be at least one and one-half ounces per square foot by passing the coated strip between coating control rolls located so as to deliver the strip upwardly from the molten bath, the exiting strip and the coating control rolls forming a crevice located on a face of the strip and containing a bead of molten metal, and

preventing draping of the molten metal coating on the strip after passage of the strip through the coating control rolls without changing the coating weight by

15

20

30

35

40

contacting the surface of the bead of molten metal with an ignited combustible gas along substantially the entire length of the bead, with the direction and velocity of the burning gas being such that the gas exerts substantially no force on the major portion of the length of the bead.

2. In continuous strip-steel hot-dip metal coating where-in a heavy galvanize coating weight is applied such that draping of the molten galvanize coating on the strip would normally occur, a method for preventing such draping of the molten coating comprising the steps of:

applying a galvanize coating to the continuous strip steel by passing the strip upwardly through a molten metal bath,

controlling the weight of the galvanize coating to be at least one and one-half ounces per square foot by passing the coated strip between coating control rolls located so as to deliver the strip upwardly from the molten bath, the exiting strip and the coating control rolls forming a crevice located on a face of the strip and containing a bead of molten metal, and preventing draping of the molten metal coating on the strip after passage of the strip through the coating control rolls without changing the coating weight by contacting the surface of the bead of molten metal with an ignited combustible gas along substantially the entire length of the bead, with the direction of flow of the burning gas being substantially parallel to the length of the bead along the major portion of the length of the bead whereby the burning gas exerts substantially no force on the major portion of the length of the bead.

#### References Cited in the file of this patent

#### UNITED STATES PATENTS

- |           |                     |               |
|-----------|---------------------|---------------|
| 2,034,348 | Lytle               | Mar. 17, 1936 |
| 2,708,171 | Inglefield          | May 10, 1955  |
| 2,894,856 | Schwendemann et al. | July 14, 1959 |
| 2,992,941 | Whitley et al.      | July 18, 1961 |